# EUROPEAN PATENT SPECIFICATION

(11) **EP 1 309 756 B1**
(45) Date of publication and mention of the grant of the patent: **13.06.2012**
(21) Application number: 01958739.3
(22) Date of filing: 02.08.2001
(51) Int. Cl.: D21H 21/16, D21H 23/76

(54) **PROCESS FOR SIZING PAPER**
VERFAHREN ZUR PAPIERLEIMUNG
PROCEDE DE COLLAGE DE PAPIER

(30) Priority: 07.08.2000 EP 00850135; 07.08.2000 EP 00850136; 07.08.2000 EP 00850137; 16.11.2000 EP 00850195
(43) Date of publication of application: 14.05.2003
(73) Proprietor: Akzo Nobel N.V., 6800 SB Arnhem (NL); Eka Chemicals AB, 445 80 Bohus (SE)
(72) Inventor: LINDGREN, Erik, S-445 34 Bohus (SE); FRÖLICH, Sten, S-436 39 Askim (SE); PERSSON, Michael, S-421 65 Västra Frölunda (SE)
(74) Representative: Alferink, Petrus J.T.
(86) International application number: PCT/SE2001/001699
(87) International publication number: WO 2002/012623

(56) References cited:
- EP-A- 0 056 876
- WO-A-98/33979
- US-A- 6 001 166
- US-A- 6 074 468

## Description

The present invention refers to a process for sizing paper which comprises adding to a suspension containing cellulosic fibres, and optional fillers, an anionic or cationic sizing dispersion, and a sizing promoter comprising a cationic organic polymer having one or more aromatic groups; and an anionic polymer having one or more aromatic groups being a step-growth polymer, a polysaccharide and a naturally occurring aromatic polymer, forming and draining the obtained suspension, wherein the sizing dispersion and sizing promoter are added separately to the aqueous suspension.

### Background

Dispersions or emulsions of sizing agents are used in papermaking in order to give paper and paper board improved resistance to wetting and penetration by various liquids. The sizing dispersions are usually added to an aqueous suspension containing cellulosic fibres, optional fillers and various additives. The aqueous suspension is fed into a headbox ejecting the suspension onto a wire where a wet web of paper is formed. To the suspension is further commonly added compounds such as starches and microparticulate materials which facilitate the dewatering of the suspension on the wire. The water drained from the wire, referred to as white water, is usually partly recirculated in the papermaking process. The cellulosic suspension contains a certain amount of non-fibrous material, for example fillers, charged polymers, sizing agents and various charged contaminants, i.e. anionic trash, electrolytes, colloidal substances, etc.. The non-fibrous material has an influence on the sizing efficiency and commonly impairs the sizing efficiency. High amounts of charged compounds such as high contents of salts in the suspension renders a suspension which is increasingly difficult to size, i.e. to obtain a paper with satisfactory sizing properties. Other compounds contained in the suspension which deteriorates sizing are various lipophilic wood extractives which may come from recycled fibres and mechanical pulps. An increased amount of added sizing agent often improve sizing, however, leading to higher costs as well an increased accumulation of sizing agents in the white water. The accumulation of non-fibrous material as well as any other component present in the suspension will be even more pronounced in mills where white water is extensively recirculated with the introduction of only low amounts of fresh water into the papermaking process. Thus, it is an objective of the present invention to further improve sizing. Another objective of the present invention is to improve sizing when sizing aqueous cellulosic containing suspensions having high conductivity ans/or high amounts of lipophilic wood extractives. Yet further objectives will appear hereinafter.

US 6001166 refers to aqueous alkyl diketen dispersions containing cationic starch and anionic dispersants such as lignin sulphonic acids, condensates of naphthalenesulphonic acid and formaldehyde.

WO 0023851 relates to anionic and cationic sizing dispersions containing ketene dimers and at least an antonic dispersing agent.

EP 984101 discloses sizing compositions comprising ketene dimers or acid anhydrides and a complexing agent selected from aminopolycarboxylic acids, N-bis- or tris-((1.2-dicraboxylethoxy)ethyl)amine and phosphonic acids. US 5972064 refers to sizing compositions comprising a thermoplastic resin selected from the group consisting of thermoplastic resins, thermoplastic hydrocarbon resins, thermoplastic polyamides and thermoplastic amide waxes.

US 5595829 discloses a paper making process comprising forming an aqueous cellulosic paper making slurry and adding a cationic polymer and an anionic polymer to the slurry to Increase retention and/or drainage. The anionic polymer comprises a formaldehyde condensate of a naphthalene sulfonic add salt.

WO 98/33979 A discloses an aqueous dispersion containing a cellulose-reactive sizing agent. US 6074468 A relates to sizing composition comprising a thermoplastic resin, starch and surfactant EP 56676 A discloses stable dispersions of fortified rosin.

### Invention

It has been found that the invention according to.the claims surprisingly solves the problems outlined in the application. More specifically, the invention relates to a process for sizing paper which comprises adding to an aqueous suspension containing cellulosic fibres, and optional fillers, an anionic or cationic sizing dispersion, and a sizing promoter comprising a cationic organic polymer having one or more aromatic groups and an anionic polymer having one or more aromatic groups being a step-growth polymer, a polysaccharide or a naturally occuring aromatic polymer, forming and draining the obtained suspension, wherein the sizing dispersion and sizing promoter are added separately to the aqueous suspension.

### Sizing dispersion

The sizing agent comprised in the anionic or cationic sizing dispersion used in the process according to the present invention is suitably any sizing agent rendering paper or board with enhanced resistance to wetting and penetration of liquids, such as non-cellulose-reactive agents including resins, e.g. fortified and/or esterified resins, waxes, fatty acids and resin acid derivatives, e.g. fatty amides and fatty esters, e.g. glycerol triesters of natural fatty acids, and/or celulose-reactive agents. Preferably, the sizing dispersion contains cellulose-reactive sizing agents. The cellulose-reactive sizing agents comprised in the sizing dispersion can be selected from any cellulose-reactive agents known in the art. Suitably, the sizing agent is selected from hydrophobic ketene dimers, ketene multimers, acid anhydrides, organic isocyanates, carbamoyl chlorides and mixtures thereof, preferably ketene dimers and/or acid anhydrides. Suitably the ketene dimers have the general formula (I) below, wherein R¹ and R² represent saturated or unsaturated hydrocarbon groups, usually saturated hydrocarbons, the hydrocarbon groups suitably having from 8 to 38 carbon atoms, usually being straight or branched chain alkyl groups having 12 to 20 carbon atom, such as hexadecyl and octadecyl groups. The ketene dimers can be liquid at ambient temperature, i.e. at 25 °C, suitably at 20 °C. Commonly, the acid anhydrides can be characterised by the general formula (II) below, wherein R³ and R⁴ can be identical or different and represent saturated or unsaturated hydrocarbon groups suitably containing from 3 to 30 carbon atoms, or R³ and R⁴ together with the -CO-C-moiety can form a 5 to 6 membered ring, optionally being further substituted with hydrocarbon groups containing up to 30 carbon atoms. Examples of acid anhydrides which are used commercially include alkyl and alkenyl succinic anhydrides and particularly isoocta-decenyl succinic anhydride.

Suitable ketene dimers, acid anhydrides and organic isocyanates include the compounds disclosed in U.S. Pat No. 4.522,686. Examples of suitable carbamoyl chlorides include those disclosed in U.S. Pat. No. 3,887,427.

The process according to the present invention comprises adding to a suspension containing cellulosic fibres an anionic or cationic aqueous sizing dispersion, i.e. the dispersing and/or stabilising agents present in the dispersion which can be referred to as the dispersing system have an overall anionic or cationic charge, respectively. The dispersing system can include any agent facilitating the formation of a dispersion or emulsion such as dispersing and/or stabilising agents exemplified by polyeledrolytes, surfactants and electrolytes. Anionic aqueous sizing dispersions may comprise cationic compounds, i.e. cationic polyelectrolytes (cationic or amphoteric polyelectrolytes with an overall cationic charge) and/or cationic surfactants and/or any other cationic compound known to the skilled person provided that the overall charge of the dispersing system is anionic. Cationic aqueous sizing dispersions, on the other hand, can comprise anionic compounds i.e. anionic polyelectrolytes (anionic or amphoteric polyelectrolytes with an overall anionic charge) and/or anionic surfactants and/or any other anionic compound known to the skilled person provided that the overall charge of the dispersing system is anionic. The anionic or cationic charge of the sizing dispersion can be determined by means of a ZetaMaster S version PCS.

According to a preferred embodiment of the present invention the anionic or cationic sizing dispersion contains a cationic organic polymer having one or more aromatic groups or/and an antionic polymer having one or more aromatic groups. The cationic organic polymer and the anionic polymer can be any of those described hereinafter comprised in the sizing promoter.

The anionic or cationic sizing dispersion added to the suspension can have a sizing agent content from 0.1 to 50 % by weight based on total dispersion/emulsion, suitably over 20% by weight. Dispersions comprising ketene dimer sizing agents may have ketene dimer contents from 5 up to 50 % by weight based on total dispersion, preferably from 10 up to 35% by weight. Dispersions, or emulsions, comprising acid anhydride sizing agents may have acid anhydride contents from 0.1 up to 30 % by weight based on total dispersion/emulsion, suitably from 1 up to 20 % by weight. Dispersions containing non-cellulose reactive sizing agents suitably have sizing agent contents from 5 up to 50 % by weight, preferably from 10 up to 35 % by weight. If an anionic and/or a cationic polymer having one or more aromatic groups are comprised in the sizing dispersion they are suitably present in an amount of from about 0.1 % by weight up to about 15 % by weight based on sizing agent.

The amount of sizing agent added to the aqueous suspension containing cellulosic fibres can be from 0.01 to 5 % by weight, suitably from 0.05 to 1.0 % by weight, based on dry weight of cellulosic fibres and optional fillers, where the dosage is dependent on the quality of the pulp or paper to be sized, the sizing agent and the level of sizing.

According to the present invention an anionic or cationic sizing dispersion and a sizing promoter comprising a cationic organic polymer having one or more aromatic groups and an anionic polymer having one or more aromatic groups being a step-growth polymer, a polysaccharide or a naturally occurring aromatic polymer are added separately to the aqueous suspension. Although the sizing dispersion may contain the same polymers as comprised in the sizing promoter, significant improvements regarding sizing, is only observed when the sizing promoter and the sizing dispersion are added separately to the cellulosic suspension. By separate addition is meant that the sizing dispersion which may comprise any of the polymers of the sizing promoter and the sizing promoter are added at different locations to the cellulosic suspension (thin stock) or at substantially the same location but timely separated. Furthermore, the cationic organic polymer and the anionic polymer forming the sizing promoter are suitably also added separately. Preferably, the anionic polymer is added to the suspension after both the sizing dispersion and the cationic organic polymer.

According to a preferred embodiment of the present invention the process for sizing paper comprises adding to an aqueous suspension containing cellulosic fibres, and optional fillers, an anionic or cationic sizing dispersion comprising a sizing agent and an anionic polymer having one or more aromatic groups being a step-growth polymer, a polysaccharide or a naturally occurring aromatic polymer, the amount of added sizing agent to the suspension being from about 0.01 % up to about 5.0 % by weight based on dry fibres; and a sizing promoter comprising a cationic polymer having one or more aromatic groups being suitably a cationic polysaccharide or a cationic vinyl addition polymer, and an anionic polymer having one or more aromatic groups being a step-growth polymer, a polysaccharide or a naturally occurring aromatic polymer, the amount of cationic polymer added to the suspension being from about 0.001 % up to about 3.0 % by weight based on dry fibres, and the amount of anionic polymer added to the suspension being from about 0.001 % up to about 3.0 % by weight based on dry fibres, forming and draining the obtained suspension, wherein the sizing dispersion and the sizing promoter are added separately to the aqueous suspension.

According to yet another preferred embodiment of the invention the anionic or cationic sizing dispersion comprises a sizing agent, a cationic organic polymer having one or more aromatic groups, such as a cationic polysaccharide or a cationic vinyl addition polymer, and an anionic polymer having one or more aromatic groups being a step-growth polymer, a polysaccharide or a naturally occurring aromatic polymer suitably the anionic polymer being a step-growth polymer or a naturally occurring aromatic polymer.

Suitably, the cationic polymer having one or more aromatic groups is a cationic polysaccharide having the structural formula (I): wherein P is a residue of a polysaccharide; A is a chain of atoms comprising C and H atoms attaching N to the polysaccharide residue, R₁ and R₂ are each H or a hydrocarbon group, R₃ is an aromatic hydrocarbon group, n is an integer from 2 up to 300000, and X⁻ is an anionic counter ion; or vinyl addition polymer obtained by polymerising a cationic monomer or a monomer mixture comprising a cationic monomer represented by the general formula (II): wherein R₁ is H or CH₃; R₂ and R₃ are each an alkyl group having from 1 to 3 carbon atoms, A₁ is O or NH, B₁ is an alkylene group having from 2 to 8 carbon atoms or a hydroxy propylene group, Q is a substituent containing an aromatic group, and X⁻ is an anionic counterion. More preferably, the cationic polymer having one or more aromatic groups is a cationic polysaccharide having the structural formula (I): wherein P is a residue of a polysaccharide; A is a chain of atoms comprising C and H atoms attaching N to the polysaccharide residue, R₁ and R₂ are each H or a hydrocarbon group, R₃ is an aromatic hydrocarbon group, n is an integer from 2 up to 300000, and X⁻ is an anionic counter ion.

### Cationic organic polymer having one or more aromatic groups

The cationic organic polymer of the sizing promoter and suitably present in the sizing dispersion can be derived from natural or synthetic sources, and can be linear, branched or cross-linked. Preferably the cationic polymer is water-soluble or water-dispersable. Examples of suitable cationic polymers include cationic polysaccharides, e.g. starches, guar gums, celluloses, chitins, chitosans, glycans, galactans, glucans, xanthan gums, pectins, mannans, dextrins, preferably starches and guar gums, suitable starches including potato, corn, wheat, tapioca, rice, waxy maize, barley, etc.; cationic synthetic organic polymers such as cationic chain-growth polymers, e.g. cationic vinyl addition polymers like acrylate-, acrylamide- and vinylamide-based polymers, and cationic step-growth polymers, e.g. cationic polyurethanes. Cationic organic polymers selected from polysaccharides, i.e. starches , and cationic vinyl addition polymers like acrylamide-based polymers having an aromatic group are particularly preferred.

The aromatic group of the cationic organic polymer can be present in the polymer backbone or in a substituent group that is attached to the polymer backbone (main chain), preferably in a substituent group. Examples of suitable aromatic groups include aryl, aralkyl and alkaryl groups, e.g. phenyl, phenylene, naphthyl, xylylene, benzyl and phenylethyl; preferably benzyl, nitrogen-containing aromatic (aryl) groups, e.g. pyridinium and quinolinium, as well as derivatives of these groups. Examples of cationically charged groups that can be present in the cationic polymer as well as in monomers used for preparing the cationic polymer include quaternary ammonium groups, tertiary amino groups and acid addition salts thereof.

According to a preferred embodiment the cationic organic polymer having an aromatic group is selected from cationic polysaccharides. The aromatic group of the polysaccharide can be attached to a heteroatom, e.g. nitrogen or oxygen, present in the polysaccharide, the heteroatom optionally being charged, for example when it is a nitrogen. The aromatic group can also be attached to a group comprising a heteroatom, e.g. amide, ester or ether, which groups can be attached to the polysaccharide backbone(main-chain), for example via a chain of atoms. Example of suitable aromatic groups and groups comprising an aromatic group include aryl and aralkyl groups, e.g. phenyl, phenylene, naphthyl, phenylene, xylylene, benzyl and phenylethyl; nitrogen-containing aromatic (aryl) groups, e.g. pyridinium and quinolinium, as well as derivatives of these groups where one or more substituents attached to said aromatic groups can be selected from hydroxyl, halides, e.g. chloride, nitro, and hydrocarbon groups having from 1 to 4 carbon atoms

Preferably, the cationic organic polymer is selected from cationic polysaccharides having the general structural formula (I): wherein P is a residue of a polysaccharide; A is a group attaching N to the polysaccharide residue, suitably a chain of atoms comprising C and H atoms, and optionally O and/or N atoms, usually an alkylene group with from 2 to 18 and suitably 2 to 8 carbon atoms, optionally interrupted or substituted by one or more heteroatoms, e.g. O or N, e.g. an alkyleneoxy group or hydroxy propylene group (- CH₂- CH(OH) - CH₂ -); R₁ and R₂ are each H or, preferably, a hydrocarbon group, suitably alkyl, having from 1 to 3 carbon atoms, suitably 1 or 2 carbon atoms; R₃ is suitably an aromatic hydrocarbon group including aralkyl groups, e.g. benzyl and phenylethyl groups; n is an integer from about 2 to about 300,000, suitably from 5 to 200,000 and preferably from 6 to 125,000 or, alternatively, R₁, R₂ and R₃ together with N form a aromatic group containing from 5 to 12 carbon atoms; and X⁻ is an anionic counterion, usually a halide like chloride.

The aromatic group modified cationic polysaccharide can have a degree of substitution varying over a wide range; the degree of cationic substitution (DS_{c}) can be from 0,01 to 0,5, suitably from 0,02 to 0,3, preferably from 0,025 to 0,2, the degree of aromatic substitution (DS_{Ar}) can be from from 0,01 to 0,5, suitably from 0,02 to 0,3, preferably from 0,025 to 0,2, and the degree of anionic substitution (DS_{A}) can be from 0 to 0,2, suitably from 0 to 0,1, preferably from 0 to 0,05.

The polysaccharides can be prepared by subjecting a polysaccharide to cationic and aromatic modification in known manner using one or more agents containing a cationic group and/or a aromatic group, for example by reacting the agent with the polysaccharide in the presence of an alkaline substance such as an alkali metal or alkaline earth metal hydroxide. The polysaccharide to be subjected to cationic and aromatic modification can be non-ionic, anionic, amphoteric or cationic. Suitable modifying agents include non-ionic agents such as, for example aralkyl halides, e.g. benzyl chloride and benzyl bromide; the reaction products of epichlorohydrin and dialkylamines having at least one substituent comprising an aromatic group as defined above, including 3-dialkylamino-1,2-epoxypropanes; and cationic agents such as, for example, the reaction product of epichlorohydrin and tertiary amines having at least one substituent comprising an aromatic group as defined above, including alkaryldialkylamines, e.g. dimethylbenzylamine; arylamines, e.g. pyridine and quinoline. Suitable cationic agents of this type include 2,3-epoxypropyl trialkylammonium halides and halohydroxypropyl trialkylammonium halides, e.g. N-(3-chloro-2-hydroxypropyl)-N-(hydrophobic alkyl)-N,N-di(lower alkyl)ammonium chloride and N-glycidyl-N-(hydrophobic alkyl)-N,N-di(lower alkyl)ammonium chloride where the aromatic group is as defined above, notably octyl, decyl and dodecyl, and the lower alkyl is methyl or ethyl; and halohydroxypropyl-N,N-dialkyl-N-alkarylammonium halides and N-glycidyl-N-(alkaryl)-N,N-dialkylammonium chloride, e.g. N-(3-chloro-2-hydroxypropyl)-N-(alkaryl)-N,N-di(lower alkyl)ammonium chloride where the alkaryl and lower alkyl groups are as defined above, particularly N-(3-chloro-2-hydroxypropyl)-N-benzyl-N,N-dimethylammonium chloride; and N-(3-chloro-2-hydroxypropyl) pyridinium chloride. Generally, when using a non-ionic aromatic agent, the polysaccharide is suitably rendered cationic by using any of the cationic agents known in the art before or after the hydrophobic modification. Examples of suitable cationic and/or aromatic modifying agents, aromatic group modified polysaccharides and methods for their preparation include those described in U.S. Patent Nos. 4,687,519 and 5,463,127; International Patent Application WO 94/24169, European Patent Application No. 189 935; and S.P. Patel, R.G. Patel and V.S. Patel, Starch/Stärke, 41 (1989), No. 5, pp. 192-196.

According to yet another preferred embodiment the cationic organic polymer is selected from homopolymers and copolymers prepared from one or more monomers comprising at least one monomer having an aromatic group, suitably an ethylenically unsaturated monomer. The synthetic polymer may be branched linear or branched. The aromatic group of the synthetic polymer can be present in the polymer backbone or, preferably, it can be a pendant group attached to or extending from the polymer backbone or be present in a pendent group that is attached to or extending from polymer backbone. Suitable aromatic (aryl) groups include those comprising a phenyl group, optionally substituted, a phenylene group, optionally substituted, and a naphthyl group, optionally substituted, for example groups having the general formulae -C₆H₅, -C₆H₄-, -C₆H₃-, and -C₆H₂-, e.g. in the form of phenylene (-C₆H₄-), xylylene (-CH₂-C₆H₄-CH₂-), phenyl (-C₆H₅), benzyl (-CH₂-C₆H₅), phenethyl (-CH₂CH₂-C₆H₅), and substituted phenyl (for example -C₆H₄-Y, -C₆H₃Y₂, and -C₆H₂Y₃) where one or more substituents (Y) attached to the phenyl ring can be selected from hydroxyl, halides, e.g. chloride, nitro, and hydrocarbon groups having from 1 to 4 carbon atoms.

Preferably, the cationic polymer is a vinyl addition polymer. The term "vinyl addition polymer" as used herein, refers to a polymer prepared by addition polymerisation polymerization of one or more vinyl monomers or ethylenically unsaturated monomers which include, for example, acrylamide-based and acrylate-based monomers. Suitably, the cationic polymer is selected from cationic vinyl addition polymers obtained by polymerising a cationic monomer or a monomer mixture comprising a cationic monomer represented by the general formula (II): wherein R₁ is H or CH₃; R₂ and R₃ are each or, preferably, an alkyl group having from 1 to 3 carbon atoms, usually 1 to 2 carbon atoms; A₁ is O or NH; B₁ is an alkylene group having from 2 to 8 carbon atoms, suitably from 2 to 4 carbon atoms, or a hydroxy propylene group; Q is a substituent containing an aromatic group, suitably a phenyl or substituted phenyl group, which can be attached to the nitrogen by means of an alkylene group usually having from 1 to 3 carbon atoms, suitably 1 to 2 carbon atoms, and preferably Q is a benzyl group (- CH₂- C₆H₅); and X⁻ is an anionic counterion, usually a halide like chloride. Examples of suitable monomers represented by the general formula (II) include quaternary monomers obtained by treating dialkylaminoalkyl (meth)acrylates, e.g. dimethylaminoethyl (meth)-acrylate, diethylaminoethyl (meth)acrylate and dimethylaminohydroxypropyl (meth)acrylate, and dialkylaminoalkyl (meth)acrylamides, e.g. dimethylaminoethyl (meth)acrylamide, diethylaminoethyl (meth)acrylamide, dimethylaminopropyl (meth)acrylamide, and diethylaminopropyl (meth)acrylamide, with benzyl chloride. Preferred cationic monomers of the general formula (II) include dimethylaminoethylacrylate benzyl chloride quaternary salt and dimethylaminoethylmethacrylate benzyl chloride quaternary salt.

The cationic vinyl addition (synthetic cationic) polymer can be a homopolymer prepared from a cationic monomer having an aromatic group or a copolymer prepared from a monomer mixture comprising a cationic monomer having an aromatic group and one or more copolymerizable monomers. Suitable copolymerizable non-ionic monomers include monomers represented by the general formula (III): wherein R₄ is H or CH₃; R₅ and R₆ are each H or a hydrocarbon group, suitably alkyl, having from 1 to 6, suitably from 1 to 4 and usually from 1 to 2 carbon atoms; A₂ is O or NH; B₂ is an alkylene group of from 2 to 8 carbon atoms, suitably from 2 to 4 carbon atoms, or a hydroxy propylene group or, alternatively, A and B are both nothing whereby there is a single bond between C and N (O=C - NR₅R₆). Examples of suitable copolymerizable monomers of this type include (meth)acrylamide; acrylamide-based monomers like N-alkyl (meth)acrylamides and N,N-dialkyl (meth)acrylamides, e.g. N-n-propylacrylamide, N-isopropyl (meth)acrylamide, N-n-butyl (meth)acrylamide, N-isobutyl (meth)acylamide and N-t-butyl (meth)acrylamide; and dialkylaminoalkyl (meth)acrylamides, e.g. dimethylaminoethyl (meth)acrylamide, diethylaminoethyl (meth)acrylamide, dimethylaminopropyl (meth)acrylamide and diethylaminopropyl (meth)acrylamide; acrylate-based monomers like dialkylaminoalkyl (meth)acrylates, e.g. dimethylaminoethyl .(meth)acrylate, diethylaminoethyl (meth)acrylate, t-butylaminoethyl (meth)acrylate and dimethylaminohydroxypropyl acrylate; and vinylamides, e.g. N-vinylformamide and N-vinylacetamide. Preferred copolymerizable non-ionic monomers include acrylamide and methacrylamide, i.e. (meth)acrylamide, and the main polymer is preferably an acrylamide-based polymer.

Suitable copolymerizable cationic monomers include the monomers represented by the general formula (IV): wherein R₇ is H or CH₃; R₈, R₉ and R₁₀ are each H or, preferably, a hydrocarbon group, suitably alkyl, having from 1 to 3 carbon atoms, usually 1 to 2 carbon atoms; A₃ is O or NH; B₃ is an alkylene group of from 2 to 4 carbon atoms, suitably from 2 to 4 carbon atoms, or a hydroxy propylene group, and X⁻ is an anionic counterion, usually methylsulphate or a halide like chloride. Examples of suitable cationic copolymerizable monomers include acid addition salts and quaternary ammonium salts of the dialkylaminoalkyl (meth)acrylates and dialkylaminoalkyl (meth)acrylamides mentioned above, usually prepared using acids like HCl, H₂O₄, etc., or quatemizing agents like methyl chloride, dimethyl sulphate, etc.; and diallyl-dimethylammonium chloride. Preferred copolymerizable cationic monomers include dimethylaminoethyl (meth)acrylate methyl chloride quaternary salt and diallyldimethyl-ammonium chloride. Copolymerizable anionic monomers like acrylic acid, methacrylic acid, various sulfonated vinyl addition monomers, etc. can also be employed and, preferably; in minor amounts.

The cationic vinyl addition polymer can be prepared from a monomer mixture generally comprising from 1 to 99 mole%, suitably from 2 to 50 mole% and preferably from 5 to 20 mole% of cationic monomer having an aromatic group, preferably represented by the general formula (II), and from 99 to 1 mole%, suitably from 98 to 50 mole%, and preferably from 95 to 80 mole% of other copolymerizable monomers which preferably comprises acrylamide or methacrylamide ((meth)acrylamide), the monomer mixture suitably comprising from 98 to 50 mole% and preferably from 95 to 80 mole% of (meth)acrylamide, the sum of percentages being 100.

The cationic polymer can also be selected from polymers prepared by condensation reaction of one or more monomers containing an aromatic group. Examples of such monomers include toluene diisocyanates, bisphenol A, phthalic acid, phthalic anhydride, etc., which can be used in the preparation of cationic polyurethanes, cationic polyamideamines, etc.

Alternatively, the organic polymer can be a polymer subjected to aromatic modification using an agent containing an aromatic group. Suitable modifying agents of this type include benzyl chloride, benzyl bromide, N-(3-chloro-2-hydroxypropyl)-N-benzyl-N,N-dimethylammonium chloride, and N-(3-chloro-2-hydroxypropyl) pyridinium chloride. Suitable polymers for such an aromatic modification include vinyl addition polymers. If the polymer contains a tertiary nitrogen which can be quatemized by the modifying agent, the use of such agents usually results in that the polymer is rendered cationic. Alternatively, the polymer to be subjected to aromatic modification can be cationic, for example a cationic vinyl addition polymer.

Usually the charge density of the vinyl addition polymer is within the range of from 0.1 to 6.0 meqv/g of dry polymer, suitably from 0.2 to 4.0 and preferably from 0.5 to 3.0.
The weight average molecular weight of synthetic polymers is usually at least about 500,000, suitably above about 1,000,000 and preferably above about 2,000,000. The upper limit is not critical; it can be about 50,000,000, usually 30,000,000 and suitably 25,000,000.

### Anionic polymer having one or more aromatic groups

The anionic polymer having an aromatic group comprised in the sizing promoter and optionally comprised in the sizing dispersion of the present invention is a step-growth polymer, a polysaccharide or a naturally occurring aromatic polymer. The term "step-growth polymer", as used herein, refers to a polymer obtained by step-growth polymerization, also being referred to as step-reaction polymer and step-reaction polymerization, respectively. Preferably, the anionic polymer comprised in the promoter is a step-growth polymer, a polysaccharide or a naturally occurring aromatic polymer with the proviso that the anionic polymer is not a melamine sulphonic acid condensation polymer. The anionic polymer may be a step-growth polymer or a naturally occurring aromatic polymer. The anionic polymers according to the invention can be linear, branched or cross-linked. The anionic polymer is commonly water-soluble or water-dispersable. The anionic polymer is preferably organic. Preferred anionic aromatic polymers are naphthalene sulphonate condensation polymers like condensated naphthalene sulphonate, and modified lignin polymers, e.g. lignin sulphonate.

The aromatic group of the anionic polymer can be present in the polymer backbone or in a substituent group that is attached to the polymer backbone (main chain). Examples of suitable aromatic groups include aryl, aralkyl and alkaryl groups and derivatives thereof, e.g. phenyl, tolyl, naphthyl, phenylene, xylylene, benzyl, phenylethyl and derivatives of these groups. Examples of anionically charged groups that can be present in the anionic polymer as well as in the monomers used for preparing the anionic polymer include groups carrying an anionic charge and acid groups carrying an anionic charge when dissolved or dispersed in water, the groups herein collectively being referred to as anionic groups, such as phosphate, phosphonate, sulphate, sulphonic acid, sulphonate, carboxylic acid, carboxylate, alkoxide and phenolic groups, i.e. hydroxy-substituted phenyls and naphthyls. Groups carrying an anionic charge are usually salts of an alkali metal, alkaline earth or ammonia.

Examples of suitable anionic step-growth polymerization products according to the present invention include condensation polymers, i.e. polymers obtained by step-growth condensation polymerization, e.g. condensates of an aldehyde such as formaldehyde with one or more aromatic compounds containing one or more anionic groups, specifically condensated naphthalene sulphonate type polymers, and optional other co-monomers useful in the condensation polymerization such as urea. Examples of suitable aromatic compounds containing anionic groups include phenolic and naphtholic compounds such as phenol, naphthol, resorcinol and derivatives thereof, aromatic acids and salts thereof such as phenylic, phenolic, naphthylic and naphtholic acids and salts, usually sulphonic acids and sulphonates, e.g. benzene sulphonic acid and sulphonate, xylen sulphonic acid and sulphonates, naphthalene sulphonic acid and sulphonate, phenol sulphonic acid and sulphonate.

Examples of further suitable anionic step-growth polymerization products according to the present invention include addition polymers, i.e. polymers obtained by step-growth addition polymerization, e.g. anionic polyurethanes prepared from a monomer mixture comprising aromatic isocyanates and/or aromatic alcohols. Examples of suitable aromatic isocyanates include diisocyanates, e.g. toluene-2,4- and 2,6-diisocyanates and diphenylmethane-4,4'-diisocyanate. Examples of suitable aromatic alcohols include dihydric alcohols, i.e. diols, e.g. bisphenol A, phenyl diethanol amine, glycerol monoterephthalate and trimethylolpropane monoterephthalate. Monohydric aromatic alcohols such as phenol and derivaties thereof may also be employed. The monomer mixture can also contain non-aromatic isocyanates and/or alcohols, usually diisocyanates and diols, for example any of those known to be useful in the preparation of polyurethanes. Examples of suitable monomers containing anionic groups include the monoester reaction products of triols, e.g. trimethylolethane, trimethylolpropane and glycerol, with dicarboxylic acids or anhydrides thereof, e.g. succinic acid and anhydride, terephthalic acid and anhydride, such as glycerol monosuccinate, glycerol monoterephthalate, trimethylolpropane monosuccinate, trimethylolpropane monoterephthalate, N,N-bis-(hydroxyethyl)-glycine, di-(hydroxymethyl)propionic acid, N,N-bis-(hydroxyethyl)-2-aminoethanesulfonic acid, and the like, optionally and usually in combination with reaction with a base, such as alkali metal and alkaline earth hydroxides, e.g. sodium hydroxide, ammonia or an amine, e.g. triethylamine, thereby forming an alkali metal, alkaline earth or ammonium counter-ion.

Examples of suitable anionic chain-growth polymerization products according to the invention include anionic vinyl addition polymers obtained from a mixture of vinylic or ethylenically unsaturated monomers comprising at least one monomer having an aromatic group and at least one monomer having an anionic group, usually co-polymerized with non-ionic monomers such as acrylate- and acrylamide-based monomers. Examples of suitable anionic monomers include (meth)acrylic acid and paravinyl phenol (hydroxy styrene).

Examples of suitable anionic polysaccharides include starches, guar gums, celluloses, chitins, chitosans, glycans, galactans, glucans, xanthan gums, pectins, mannans, dextrins, preferably starches, guar gums and cellulose derivatives, suitable starches including potato, com, wheat, tapioca, rice, waxy maize and barley, preferably potato. The anionic groups in the polysaccharide can be native and/or introduced by chemical treatment. The aromatic groups in the polysaccharide can be introduced by chemical methods known in the art.

Examples of suitable (modified) naturally occurring aromatic anionic polymers of this invention include Kraft lignin, such as modified lignin polymers like lignin adducts copolymerised with formaldehyde and sulphonated lignin, e.g. lignin sulphonate and tannin extracts, i.e. naturally occuring polyphenolic substances that are present in the organic extracts of bark of some wood species.

Suitably, the anionic polymer having an aromatic group is selected from step-growth polymers, polysaccharides and naturally occurring aromatic polymer. Condensated naphthalene sulphonate type polymers like condesated naphthalene sulphonate and modfied lignin polymers such as lignin sulphonates are preferred.

The weight average molecular weight of the anionic polymer can vary within wide limits dependent on, inter alia, the type of polymer used, and usually it is at least about 500, suitably above about 2,000 and preferably above about 5,000. The upper limit is not critical; it can be about 200,000,000, usually 150,000,000, suitably 100,000,000 and preferably 1,000,000.

The anionic polymer can have a degree of anionic substitution (DS_{A}) varying over a wide range dependent on, inter alia, the type of polymer used; DS_{A} is usually from 0.01 to 2.0, suitably from 0.02 to 1.8 and preferably from 0.025 to 1.5; and the degree of aromatic substitution (DS_{Q}) can be from 0.001 to 1.0, usually from 0.01 to 0.8, suitably from 0.02 to 0.7 and preferably from 0.025 to 0.5. In case the anionic polymer contains cationic groups, the degree of cationic substitution (DS_{C}) can be, for example, from 0 to 0.2, suitably from 0 to 0.1 and preferably from 0 to 0.05, the anionic polymer having an overall anionic charge. Usually the anionic charge density of the anionic polymer is within the range of from 0.1 to 6.0 meqv/g of dry polymer, suitably from 0.5 to 5.0 and preferably from 1.0 to 4.0.

The cationic organic polymer having an aromatic group and the anionic polymer having an aromatic group of the sizing promoter can be added to the aqueous suspension (stock) in any order separately from the addition of the sizing dispersion and in amounts which can vary within wide limits depending on, inter alia, type of stock, salt content, type of salts, filler content, type of filler, point of addition, etc. Generally the polymers are added in an amount that give better sizing than is obtained when not adding them and usually the cationic organic polymer is added to the stock prior to adding the anionic polymer. The cationic polymer is usually added in an amount of at least 0.001%, often at least 0.005% by weight, based on dry stock substance, whereas the upper limit is usually 3% and suitably 2.0% by weight. The anionic polymer is usually added in an amount of at least 0.001%, often at least 0.005% by weight, based on dry stock substance, whereas the upper limit is usually 3% and suitably 1.5% by weight

Apart from the cationic organic polymer and the anionic polymer the sizing promoter may contain other compounds which improve the sizing efficiency such as anionic microparticulate materials, e.g., silica-based particles and clays of smectite type, low molecular weight cationic organic polymers, aluminium compounds like alum, aluminates, aluminium chloride, aluminium nitrate and polyaluminium compounds, such as polyaluminium chlorides, polyaluminium sulphates, polyaluminium compounds containing both chloride and sulphate ions, polyaluminium silicate-sulphates and mixtures thereof, anionic vinyl addition polymers and combinations thereof.

The process of the invention is preferably used in the manufacture of paper from a suspension containing cellulosic fibers, and optional fillers, having a high conductivity. Usually, the conductivity of the stock is at least 0.20 mS/cm, suitably at least 0.5 mS/cm, preferably at least 3.5 mS/cm. Very good sizing results have been observed at conductivity levels above 5.0 mS/cm and even above 7.5 mS/cm. Conductivity can be measured by standard equipment such as, for example a WTW LF 539 instrument supplied by Christian Bemer. The values referred to above are suitably determined by measuring the conductivity of the cellulosic suspension that is fed into or present in the headbox of the paper machine or, alternatively, by measuring the conductivity of white water obtained by dewatering the suspension. High conductivity levels mean high contents of salts (electrolytes), where the various salts can be based on mono-, di- and multivalent cations like alkali metals, e.g. Na⁺ and K⁺, alkaline earths, e.g. Ca²⁺ and Mg²⁺, aluminium ions, e.g. Al³⁺, Al(OH)²⁺ and polyaluminium ions, and mono-, di- and multivalent anions like halides, e.g., Cr, sulfates, e.g. SO₄²⁻ and HSO₄⁻, carbonates, e.g. CO₃²⁻ and HCO₃⁻, silicates and lower organic acids. The invention is particularly useful in the manufacture of paper from stocks having high contents of salts of di- and multivalent cations, and usually the cation content is at least 200 ppm, suitably at least 300 ppm and preferably at least 400 ppm. The salts can be derived from the cellulosic fibres and fillers used to form the stock, in particular in integrated mills where a concentrated aqueous fibre suspension from the pulp mill normally is mixed with water to form a dilute suspension suitable for paper manufacture in the paper mill. The salt may also be derived from various additives introduced into the stock, from the fresh water supplied to the process, or be added deliberately, etc. Further, the content of salts is usually higher in processes where white water is extensively recirculated, which may lead to considerable accumulation of salts in the water circulating in the process.

The present invention further encompasses papermaking processes where white water is extensively recirculated (recycled), i.e. with a high degree of white water closure, for example where from 0 to 30 tons of fresh water are used per ton of dry paper produced, usually less than 20, suitably less than 15, preferably less than 10 and notably less than 5 tons of fresh wafer per ton of paper. Recirculation of white water obtained in the process suitably comprises mixing the white water with cellulosic fibres and/or optional fillers to form a suspension to be sized; preferably it comprises mixing the white water with a suspension containing cellulosic fibres, and optional fillers, before the suspension enters the forming wire for sizing.

Further additives which are conventional in papermaking can of course be used in combination with the additives according to the invention, such as, for example, additional dry strength agents, wet strength agents. The cellulosic suspension, or stock, can also contain mineral fillers of conventional types such as, for example, kaolin, china clay, titanium dioxide, gypsum, talc and natural and synthetic calcium carbonates such as chalk, ground marble and precipitated calcium carbonate.

The process of this invention is used for the production of paper. The term "paper", as used herein, of course include not only paper and the production thereof, but also other sheet or web-like products, such as for example board and paperboard, and the production thereof. The process can be used in the production of paper from different types of suspensions of cellulose-containing fibres and the suspensions should suitably contain at least 25% by weight and preferably at least 50% by weight of such fibres, based on dry substance. The suspensions can be based on fibres from chemical pulp such as sulphate, sulphite and organosolv pulps, mechanical pulp such as thermomechanical pulp, chemo-thermomechanical pulp, refiner pulp and groundwood pulp, from both hardwood and softwood, and can also be based on recycled fibres, optionally from de-inked pulps, and mixtures thereof. The invention is particularly useful in the manufacture of paper from suspensions based on pulps comprising recycled fibres and de-inked pulp, and the content of cellulosic fibres of such origin can be up to 100%, suitably from 20% to 100%.

The invention is further illustrated in the following Examples which, however, are not intended to limit the same. Parts and % relate to parts by weight and % by weight, respectively, unless otherwise stated.

In all examples hereinafter the sizing dispersion and the sizing prompter were added separately to the cellulosic suspension. Furthermore, in the case the promoter comprised more than one polymer having an aromatic group, these polymers were added separately to the suspension with respect to each other and to the dispersion.

### Example 1

The sizing performance of the process was evaluated by using the cobb 60 test.

An anionic sizing dispersion was prepared containing alkyl ketene dimer, condensated naphthalene sulphonate and di(hydrogenated tallow) dimethylammonium chloride. The sizing dispersion had an AKD content of 30% and contained 4% of di(hydrogenated tallow) dimethylammonium chloride and 6% of condensated naphthalene sulphonate based on AKD. The sizing dispersion was added to the stock in an amount of 5 kg AKD/tonne dry stock.

In test 2 the sizing promoter comprised condensated naphtalene sulphonate (available under the trade name Tamol ®) and a cationic starch with a cationic substitution DS of 0.065 regarding nitrogen containing benzyl groups. In test 1 cationic starch without aromatic groups with a cationic substitution of 0.065 and anionic inorganic silica particles provided as a sol, i.e. an anionic non-aromatic polymer, was added to the furnish.

The furnish used was based on 80 % by weight of bleached birch/pine (60/40) sulphate pulp and 20 % by weight of CaCO₃ refined to 200 CSF and containing 0.3 g/litre stock Na₂SO₄, having a conductivity of 461 µS/cm and a pH of 8,1.

### Example 2

The sizing performance of the process was evaluated (cobb 60 test) by adding the same anionic sizing dispersion as described in example 1 and a sizing promoter comprising cationic starch with a cationic substitution DS of 0.065 regarding nitrogen containing benzyl groups and anionic inorganic silica particles (test 1); and a promoter comprising condensated naphtalene sulphonate (available under the trade name Tamol ®) and a cationic starch with a cationic substitution DS of 0.065 regarding nitrogen containing benzyl groups (test 2). However, calcium chloride was added to the furnish to adjust the conductivity to 5000 µS/cm thereby simulating a furnish having high conductivity.

### Example 3

The sizing performance was evaluated using a cationic sizing dispersion which contained 15 % of alkyl ketene dimer, 2 % of cationic starch and 0.6% of sodium lignosulphonte, based on AKD. The components and added amount of components comprised in the sizing promoter, apparent from table 3, included condensated naphtalene sulphonate, cationic starch without aromatic groups having a DS of 0.065, cationic starch containing aromatic groups having a DS of 0.065 and anionic inorganic silica particles provided as a sol. The stock used was that of example 2 having a pH of 8.1 and a conductivity of 5000 µS/cm by the addition of calcium chloride to the stock.

### Example 4

An anionic sizing dispersion was prepared containing 8,9 % of a commercial alkyl ketene dimer, 0,89 % of an aromat substituted cationic starch having a DS of 0,065 containing benzyl groups, and 0,22 % of condensated naphthalene sulphonate available under the trade name Tamol ®. The anionic dispersion was added in an amount of 0,0115% (dry base) based on the ketene dimer to a cellulosic suspension (dry base) containing 30% Pine, 30% Bee, 40% Eucaluptus, and 15% of precipitated CaCO₃. The conductivity of the suspension was 500 µS/cm. To the suspension was also added a sizing promoter containing benzyl substituted starch having a DS of 0.065 and condensated naphtalene sulphonate available under the trade name Tamol ® (test 2).

To the same suspension was also added the same anionic dispersion. However, the sizing promoter added to the suspension contained no aromatic polymers. The sizing promoter contained cationic starch with a DS of 0.065 having no aromatic groups and anionic inorganic silica particles provided as a sol (test 1). The amounts of polymers of the promoter and sizing agent (AKD) of the dispersion are given in table 4.

### Example 5

In this example the same dispersion and sizing promoters were used as in example 2 except that the conductivity of the suspension was 5000 µS/cm.

The amounts of polymers of the promoter and sizing agent (AKD) of the dispersion are given in table 5.

### Example 6

The sizing performance of the process was evaluated by using the Cobb 60 test. An anionic sizing dispersion was prepared containing alkyl ketene dimer, condensed naphtalene sulphonate and di(hydrogenated tallow) dimethylammonium chloride. The sizing dispersion had an AKD content of 30% and contained 4% of di(hydrogenated tallow) dimethylammunium chloride and 6% of condensed naphtalene sulphonate, based on AKD. The sizing dispersion was added in an amount of 0.3 kg AKD/ tonne of dry stock.

A cationic starch with a cationic substitution DS of 0.065 regarding nitrogen containing benzylgruops and a starch with a cationic substitution DS of 0.065 were used in a combination of a condensed naphtalene sulphonate and a melamin sulphonate, respectively.

The furnish used was based on 80% birch/pine (60/40) sulphate pulp and 20% by weight oc CaCO₃ , refinded to 200 CSF and containing 0.3 g/litre stock giving a conductivity of 555µS/cm and a pH 8,22.

## Claims

1. A process for sizing paper which comprises adding to an aqueous suspension containing cellulosic fibres, and optional fillers,
(i) an anionic or cationic sizing dispersion; and
(ii) a sizing promoter comprising a cationic organic polymer having one or more aromatic groups, and an anionic polymer having one or more aromatic groups, the anionic polymer being a step-growth polymer, a polysaccharide or a naturally occurring aromatic polymer,
forming and draining the obtained suspension, wherein the sizing dispersion and sizing promoter are added separately to the aqueous suspension.

2. The process according to claim 1, wherein the cationic organic polymer and the anionic polymer comprised in the sizing promoter are added separately to the aqueous suspension.

3. The process according to claim 1, wherein the anionic polymer having an aromatic group comprised in the sizing promoter is added to the aqueous suspension after both the sizing dispersion and the cationic organic polymer having an aromatic group comprised in the sizing promoter.

4. The process according to any of the preceding claims, wherein the cationic organic polymer is a cationic polysaccharide or a cationic vinyl addition polymer.

5. The process according to any of the preceding claims, wherein the cationic organic polymer is a cationic polysaccharide having the structural formula (I): wherein P is a residue of a polysaccharide; A is a chain of atoms comprising C and H atoms attaching N to the polysaccharide residue, R₁ and R₂ are each H or a hydrocarbon group, R₃ is an aromatic hydrocarbon group, n is an integer from 2 up to 300000, and X⁻ is an anionic counter ion; and/or vinyl addition polymers obtained by polymerising a cationic monomer or a monomer mixture comprising a cationic monomer represented by the general formula (II): wherein R₁ is H or CH₃; R₂ and R₃ are each an alkyl group having from 1 to 3 carbon atoms, A₁ is O or N H, B₁ is an alkylene group having from 2 to 8 carbon atoms or a hydroxy propylene group, Q is a substituent containing an aromatic group, and X⁻ is an anionic counterion.

6. The process according to claim 1, wherein the cationic organic polymer is selected from cationic polysaccharides.

7. The process according to claim 1, wherein the cationic organic polymer is selected from cationic starch.

8. The process according to claim 1, wherein the cationic polymer is selected from cationic polysaccharides having the structural formula (I): wherein P is a residue of a polysaccharide; A is a chain of atoms comprising C and H atoms attaching N to the polysaccharide residue, R₁ and R₂ are each H or a hydrocarbon group, R₃ is an aromatic hydrocarbon group, n is an integer from 2 up to 300000, and X⁻ is an anionic counter ion.

9. The process according to claim 8, wherein A is an alkylene group with from 2 to 18 carbon atoms, optionally interrupted or substituted by one or more heteroatoms; R₁ and R₂ are each H or an alkyl group having from 1 to 3 carbon atoms; R₃ is a benzyl or phenylethyl group.

10. The process according to any of the preceding claims, wherein the anionic polymer is a step-growth polymer or a naturally occurring aromatic polymer.

11. The process according to any of the claims 1 to 9, wherein the anionic polymer is a naphthalene sulphonate condensation polymer or modified lignin polymer.

12. The process according to any of the claims 1 to 9, wherein the anionic polymer is condesated naphthalene sulphonate or lignin sulphonate.

13. The process according to any of the preceding claims, wherein the sizing dispersion comprises cellulose-reactive sizing agents.

14. The process according to any of the preceding claims, wherein the sizing dispersion comprises cellulose-reactive sizing agents selected from ketene-dimers and/or acid anhydrides.

15. The process according to any of the preceding claims, wherein the sizing dispersion comprises cellulose-reactive sizing agents selected from acid anhydrides.

## Patentansprüche

1. Ein Verfahren zur Papierleimung, welches die Zugabe zu einer wässrigen Suspension enthaltend cellulosehaltige Fasern und optionale Füllstoffe von
(i) einer anionischen oder kationischen Leimungsdispersion; und
(ii) eines Leimungsbeschleunigers, umfassend ein kationisches organisches Polymer mit einer oder mehreren aromatischen Gruppen und ein anionisches Polymer mit einer oder mehreren aromatischen Gruppen, wobei das anionische Polymer ein Stufenwachstumspolymer, ein Polysaccharid oder ein natürlich vorkommendes aromatisches Polymer ist,
das Formgeben und das Entwässern der erhaltenen Suspension umfasst, wobei die Leimungsdispersion und der Leimungsbeschleuniger der wässrigen Suspension separat zugegeben werden.

2. Das Verfahren gemäß Anspruch 1, wobei das kationische organische Polymer und das anionische Polymer, welche in dem Leimungsbeschleuniger enthalten sind, separat zu der wässrigen Suspension zugegeben werden.

3. Das Verfahren gemäß Anspruch 1, wobei das anionische Polymer mit einer aromatischen Gruppe, welches in dem Leimungsbeschleuniger enthalten ist, nach der Leimungsdispersion und dem kationischen organischen Polymer mit einer aromatischen Gruppe, welches in dem Leimungsbeschleuniger enthalten ist, zu der wässrigen Suspension gegeben wird.

4. Das Verfahren gemäß einem der vorstehenden Ansprüche, wobei das kationische organische Polymer ein kationisches Polysaccharid oder ein kationisches Vinyladditionspolymer ist.

5. Das Verfahren gemäß einem der vorstehenden Ansprüche, wobei das kationische organische Polymer ein kationisches Polysaccharid der Strukturformel (I): wobei P ein Rest eines Polysaccharids ist; A eine Kette von Atomen umfassend C und H Atome, welche N an den Polysaccharidrest anbindet, ist, R₁ und R₂ jeweils H oder ein Kohlenwasserstoffrest sind, R₃ ein aromatischer Kohlenwasserstoffrest ist, n eine ganze Zahl von 2 bis 300000 ist, und X⁻ ein anionisches Gegenion ist; und/oder Vinyladditionspolymere erhalten durch Polymerisieren eines kationischen Monomers oder eines Monomergemischs umfassend ein kationisches Monomer, dargestellt durch die allgemeine Formel (II), ist: wobei R₁ die Bedeutung H oder CH₃ hat; R₂ und R₃ jeweils ein Alkylrest mit 1 bis 3 Kohlenstoffatomen sind, A₁ die Bedeutung O oder NH hat, B₁ ein Alkylenrest mit 2 bis 8 Kohlenstoffatomen oder eine Hydroxypropylengruppe ist, Q ein Substituent enthaltend einen aromatischen Rest ist, und X⁻ ein anionisches Gegenion ist.

6. Das Verfahren gemäß Anspruch 1, wobei das kationische organische Polymer aus kationischen Polysacchariden ausgewählt ist.

7. Das Verfahren gemäß Anspruch 1, wobei das kationische organische Polymer aus kationischer Stärke ausgewählt ist.

8. Das Verfahren gemäß Anspruch 1, wobei das kationische Polymer aus kationischen Polysacchariden der Strukturformel (I) ausgewählt ist: wobei P ein Rest eines Polysaccharids ist; A eine Kette von Atomen umfassend C und H Atome, welche N an den Polysaccharidrest anbindet, ist, R₁ und R₂ jeweils H oder ein Kohlenwasserstoffrest sind, R₃ ein aromatischer Kohlenwasserstoffrest ist, n eine ganze Zahl von 2 bis 300000 ist, und X⁻ ein anionisches Gegenion ist.

9. Das Verfahren gemäß Anspruch 8, wobei A ein Alkylenrest mit 2 bis 18 Kohlenstoffatomen ist, optional unterbrochen durch oder substituiert mit ein(em) oder mehrere(n) Heteroatomen; R₁ und R₂ jeweils H oder ein Alkylrest mit 1 bis 3 Kohlenstoffatomen sind; R₃ eine Benzyl- oder Phenylethylgruppe ist.

10. Das Verfahren gemäß einem der vorstehenden Ansprüche, wobei das anionische Polymer ein Stufenwachstumspolymer oder ein natürlich vorkommendes aromatisches Polymer ist.

11. Das Verfahren gemäß einem der Ansprüche 1 bis 9, wobei das anionische Polymer ein Naphthalinsulfonat-Kondensationspolymer oder ein modifiziertes Ligninpolymer ist.

12. Das Verfahren gemäß einem der Ansprüche 1 bis 9, wobei das anionische Polymer kondensiertes Naphthalinsulfonat oder Ligninsulfonat ist.

13. Das Verfahren gemäß einem der vorstehenden Ansprüche, wobei die Leimungsdispersion Cellulose-reaktive Leimungsmittel umfasst.

14. Das Verfahren gemäß einem der vorstehenden Ansprüche, wobei die Leimungsdispersion Cellulose-reaktive Leimungsmittel ausgewählt aus Ketendimeren und/oder Säureanhydriden umfasst.

15. Das Verfahren gemäß einem der vorstehenden Ansprüche, wobei die Leimungsdispersion Cellulose-reaktive Leimungsmittel ausgewählt aus Säureanhydriden umfasst.

## Revendications

1. Procédé de collage de papier qui comprend l'addition à une suspension aqueuse contenant des fibres cellulosiques, et des charges optionnelles,
(i) d'une dispersion de collage anionique ou cationique ; et
(ii) d'un agent de collage comprenant un polymère organique cationique comportant un ou plusieurs groupes aromatiques, et un polymère anionique comportant un ou plusieurs groupes aromatiques, le polymère anionique étant un polymère à croissance par étapes, un polysaccharide ou un polymère aromatique naturel,
la formation et le drainage de la suspension obtenue, dans lequel la dispersion de collage et l'agent de collage sont ajoutés séparément à la suspension aqueuse.

2. Procédé selon la revendication 1, dans lequel le polymère organique cationique et le polymère anionique contenus dans l'agent de collage sont ajoutés séparément à la suspension aqueuse.

3. Procédé selon la revendication 1, dans lequel le polymère anionique comportant un groupe aromatique contenu dans l'agent de collage est ajouté à la suspension aqueuse après la dispersion de collage et le polymère organique cationique comportant un groupe aromatique contenu dans l'agent de collage.

4. Procédé selon l'une quelconque des revendications précédentes, dans lequel le polymère organique cationique est un polysaccharide cationique ou un polymère d'addition vinylique cationique.

5. Procédé selon l'une quelconque des revendications précédentes, dans lequel le polymère organique cationique est un polysaccharide cationique présentant la formule structurale (I) : dans laquelle P représente un résidu de polysaccharide ; A représente une chaîne d'atomes comprenant des atomes de C et d'H reliant l'atome de N au résidu de polysaccharide, R₁ et R₂ représentent chacun un atome d'H ou un groupe hydrocarbure, R₃ représente un groupe hydrocarbure aromatique, n représente un nombre entier de 2 à 300 000, et X⁻ représente un contre-ion anionique, et/ou des polymères d'addition vinylique obtenus en polymérisant un monomère cationique ou un mélange de monomères comprenant un monomère cationique représenté par la formule générale (II) : dans laquelle R₁ représente un atome d'H ou un groupe CH₃ ; R₂ et R₃ représentent chacun un groupe alkyle comportant de 1 à 3 atomes de carbone, A₁ représente un atome d'O ou un groupe NH, B₁ représente un groupe alkylène comportant de 2 à 8 atomes de carbone ou un groupe hydroxypropylène, Q représente un substituant contenant un groupe aromatique, et X⁻ représente un contre-ion anionique.

6. Procédé selon la revendication 1, dans lequel le polymère organique cationique est choisi parmi les polysaccharides cationiques.

7. Procédé selon la revendication 1, dans lequel le polymère organique cationique est choisi parmi un amidon cationique.

8. Procédé selon la revendication 1, dans lequel le polymère cationique est choisi parmi les polysaccharides cationiques présentant la formule structurale (I) : dans laquelle P représente un résidu de polysaccharide ; A représente une chaîne d'atomes comprenant des atomes de C et d'H reliant l'atome de N au résidu de polysaccharide, R₁ et R₂ représentent chacun un atome d'H ou un groupe hydrocarbure, R₃ représente un groupe hydrocarbure aromatique, n représente un nombre entier de 2 à 300 000, et X⁻ représente un contre-ion anionique.

9. Procédé selon la revendication 8, dans lequel A représente un groupe alkylène comportant de 2 à 18 atomes de carbone, optionnellement interrompus ou substitués par un ou plusieurs hétéroatomes ; R₁ et R₂ représentent chacun un atome d'H ou un groupe alkyle comportant de 1 à 3 atomes de carbone ; R₃ représente un groupe benzyle ou phényléthyle.

10. Procédé selon l'une quelconque des revendications précédentes, dans lequel le polymère anionique est un polymère à croissance par étapes ou un polymère aromatique naturel.

11. Procédé selon l'une quelconque des revendications 1 à 9, dans lequel le polymère anionique est un polymère de condensation de type sulfonate de naphtalène ou un polymère à base de lignine modifiée.

12. Procédé selon l'une quelconque des revendications 1 à 9, dans lequel le polymère anionique est un sulfonate de naphtalène condensé ou un sulfonate de lignine.

13. Procédé selon l'une quelconque des revendications précédentes, dans lequel la dispersion de collage comprend des agents de collage réactifs avec la cellulose.

14. Procédé selon l'une quelconque des revendications précédentes, dans lequel la dispersion de collage comprend des agents de collage réactifs avec la cellulose choisis parmi les dimères de cétène et/ou les anhydrides d'acide.

15. Procédé selon l'une quelconque des revendications précédentes, dans lequel la dispersion de collage comprend des agents de collage réactifs avec la cellulose choisis parmi les anhydrides d'acide.
